

# UNITED STATES PATENT OFFICE.

WILHELM EBERLE, OF ETTLINGEN, NEAR KARLSRUHE, GERMANY.

## BLASTING-POWDER.

No. 910,365.

Specification of Letters Patent.

Patented Jan. 19, 1909.

Application filed August 12, 1908. Serial No. 448,233.

*To all whom it may concern:*

Be it known that I, WILHELM EBERLE, a subject of the German Emperor, residing at Ettingen, near Karlsruhe, Baden, Germany, have invented certain new and useful Improvements in Blasting-Powder, of which the following is a specification.

The subject-matter of the present invention is an agent for blasting rocks and the like, and an important object is to provide an agent which has the advantage that when comparatively small charges are used, it breaks rock into pieces having straight surfaces, without the rocks or the like being appreciably splintered or shivered.

As compared with the agent which has almost solely come into use heretofore in practice, namely blasting powder, the blasting agent according to the present invention has the further advantage that the intended object can be attained by one single blasting operation, whereas when blasting powder is used in a bore-hole of the same size, frequently three to four blasting operations were required. Further, the new agent is superior to blasting powder with regard to danger, since it can be rammed into the bore-hole by means of an iron rod, for example, which operation would cause an explosion if blasting powder were used.

The blasting agent according to the present invention contains saltpeter, sulfur, charcoal and horse-dung in the form of dust or powder, in the proportion of about 12:3:1:1 parts by weight respectively. As is known, blasting agents made of like or similar substances have been employed for similar purposes, as may be seen from the British Patent Specifications No. 13822 of the year 1897 and No. 18516 of the year 1899, as well as from the American Patent Specification No. 757,693, but the agent according to the present invention has various advantages as

compared with these known agents, as is explained above and hereafter. Namely, experiments have shown that the blasting agents described in the above mentioned patent specifications were either quite ineffective and were hurled out from the bore-hole after ignition, and were thus inoperative, or they only produced a very small effect.

The astonishing effect obtained with the blasting agent according to the present invention is apparently attributable to its special composition which is such that an especially favorable combustion and development of gases takes place for the required purpose.

For making the blasting agent, fresh horse-dung which is thoroughly dried in the air and disintegrated so as to form a fine meal or powder is employed and is mixed evenly with the other materials in the above mentioned proportions. Now I am aware that saltpeter, sulfur, carbon and horse-dung have severally been used heretofore for making various blasting agents, and I therefore do not claim an agent consisting of this combination of substances broadly. By mixing these materials in certain definite proportions, however, it is found that very considerably improved results are obtained, and

What I claim is:—

The herein described blasting agent consisting of saltpeter, sulfur, carbon, and horse-dung in the form of dust, in the proportions of twelve to three to one to one parts by weight respectively, substantially as described.

In testimony whereof, I affix my signature in the presence of two witnesses.

WILHELM EBERLE.

Witnesses:

RAY SIGSBEE,  
Jos. H. LEUTE.